

June 3, 1969

H. I. MOSS ET AL

3,448,184

METHOD FOR PRESSING PARTICULATE MATERIAL

Filed April 8, 1966



INVENTORS  
HERBERT I. MOSS &  
WILLIAM P. STOLLAR

BY Glenn A. Bernstein  
Attorney

## 1

3,448,184

## METHOD FOR PRESSING PARTICULATE MATERIAL

Herbert Irwin Moss, Yardley, Pa., and William Porter Stollar, Edison, N.J., assignors to Radio Corporation of America, a corporation of Delaware

Filed Apr. 8, 1966, Ser. No. 541,325  
Int. Cl. B29f 5/02

U.S. Cl. 264—125

5 Claims

## ABSTRACT OF THE DISCLOSURE

In a method for pressing solid particulate material, the material to be pressed is placed in a die comprising a support sleeve, which supports a liner within the sleeve. Pressure rams are adapted to move axially within the die so as to compress the material therein. Prior to and during compression of the material within the die, a force is applied to the die liner in the axial direction. This axial force permits the application of increased pressure upon the material to be compressed without failure of the die liner.

This invention relates to a method for pressing particulate materials, and particularly, to a method for compacting powders into unitary bodies. Such methods may, e.g., be used in the manufacture of polycrystalline ferrite bars, infrared transmission windows and semiconductor bodies.

To obtain uniformly dense compacted masses of powders by pressing, high pressures are essential. Present pressing procedures utilize a die and ram assembly in which the die is comprised of a support sleeve and a die liner made of a high lubricity material, such as graphite. The material to be pressed is placed in the die liner and compressed between two rams. One difficulty with present pressing procedures is mechanical failure of the die liner at relatively low pressures. This failure causes the die liner to crumble and to be forced out of its support sleeve resulting in the loss of the material being compressed.

An object of this invention is to provide a new and improved method for pressing solid materials.

Another object of this invention is to provide a method capable of pressing solid materials at greater than normal pressures.

A further object is to provide a method of pressing materials in a die using graphite liners at pressures well beyond that which graphite liners normally fail.

An additional object is to provide a method of compacting and sintering powders of inorganic compounds.

The novel method may be used in pressing techniques in which a quantity of powder is pressed with a ram or rams in a die comprised of a die liner within a support sleeve. The support sleeve provides support for the die liner in the radial direction, the radial direction being normal to the direction of movement of the rams in the die.

One feature characterizing the novel method is that axial pressure is applied to the die liner while the material is being pressed within the die liner. As used herein, the axial direction is parallel to the direction of movement of the rams in the die. By applying axial pressure to the die liner while pressing the material within the liner, forces are created which reduce the stress within the liner, thereby allowing much higher pressures to be applied to the material to be compressed before the die fails.

The invention is described below in more detail with reference to the drawings in which:

FIG. 1 is a front elevational, partially sectional view of a prior-art die and ram assembly illustrating some of the forces on the die liner.

## 2

FIG. 2 is a front elevational, partially sectional view of a die and ram assembly that may be used in practicing the novel method disclosed herein.

Similar reference numerals are used for similar structural elements in the drawings.

The prior-art die and ram assembly illustrated in FIG. 1 is comprised of a die 1 and lower and upper rams 2 and 3 adapted to move within the die. The die 1 is comprised of a die liner 4 within a support sleeve 5. The support sleeve 5 supports the die liner 4 when outwardly directed radial pressure is present on the liner 4.

In operation, the lower ram 2 is placed in the liner 4. A quantity of material 6 to be compressed is inserted into the liner 4. The upper ram 3 is then lowered into the liner 4 and the rams 2 and 3 are moved toward each other so as to compress the material 6 between them. During compression of the material 6, the rams exert an applied force  $F_1$  on said material 6. This applied force  $F_1$  creates an outwardly directed essentially radial force  $F_2$  within the material 6 which causes stresses on the liner 4. The magnitude of the radial force  $F_2$  for a given applied force  $F_1$  depends on the plasticity of the material 6 to be compressed. When the applied force  $F_1$  reaches some critical value, depending on the composition and dimensions of the liner 4 and on the material 6 being compressed, the liner 4 fails by crumbling in a ring like volume and is forced out of the support sleeve 5. It is believed that this is due to a combination of initial radial compressive failure of the liner 4 due to the radial force  $F_2$ , followed by axial tensile failure due to the development of axial components to the radial force  $F_2$ . These axial components cause the die liner 4 to separate in the area adjacent the compacted material 6 thereby forcing the liner out of the support sleeve 5. The combination of radial compressive and axial tensile failure being a catastrophic process.

The novel method essentially overcomes the problem of failure of the die liner as described above. FIG. 2 is a view of a die and ram assembly that may be used to practice the novel method of pressure compacting disclosed herein. FIG. 2 also indicates certain forces present on the die during the practice of the novel method. The assembly includes lower and upper rams 2a and 3a respectively which compress material 6a within a die 1a comprised of a die liner 4a within a support sleeve 5a. The support sleeve 5a has an inwardly projecting lip 7 on the lower portion thereof, an internally threaded upper portion 8 and a central cylindrical portion 9. The inside diameter of the upper portion 8 is greater than the inside diameter of the central cylindrical portion 9. The liner 4a has a cylindrical outer surface and fits snugly into the central cylindrical portion 9 of the support sleeve 5a and is supported thereby when an outwardly directed radial force is present on the liner 4a. The bottom of the liner 4a rests on the lip 7 of the support sleeve 5a and is supported thereby. The liner 4a has an upper portion 10 which extends above the cylindrical portion 9 and into the area of the threaded upper portion 8 of the support sleeve 5a.

The assembly includes a cylindrical plug 11 threaded on its outer cylindrical surface so as to mate with and screw into the threaded upper portion 8 of the support sleeve 5a. The plug 11 has a vertical center hole so that the upper ram 3a can fit therethrough. The lower ram 2a enters the die liner 4a through the end opposite the plug 11. A heating coil 12 around the support sleeve 5a can also be included.

In operation, the plug 11 is screwed into the threaded upper portion 8 of the support sleeve 5a so as to create a high compressive axial linear force  $F_3$  on the liner 4a in the axial direction. The axial direction, as pointed out above, is defined herein as the direction in which the rams 2a and 3a move in the die liner 4a. The lower ram 2a is then positioned in the liner 4a, and the material 6a

to be compressed is placed in the liner 4a. The upper ram 3a is then lowered into place and a compressive force  $F_1$  is applied to the material 6a by moving the rams 2a and 3a together. During compression the axial liner force  $F_3$  previously placed on the liner 4a is continued.

The liner 4a and the material 6a contained therein may be heated to any desired temperature by the heating coil 12. The heat can be applied at any stage and continued throughout the operation if desired. A thermocouple or other temperature sensitive device (not shown) can be used to control and measure the temperature.

After maintaining the pressure and temperature at prescribed magnitudes and for prescribed times dependent on the material 6a to be compressed and the desired density of the compressed material, the pressure on the material 6a is released by moving the rams 2a and 3a apart. The compressed material 6a is then removed from the die 1a. The compressive axial liner force,  $F_3$ , on the liner 4a may also be released.

It has been found that the application of the axial liner force  $F_3$  on the die liner 4a as described above permits much greater than normal force to be applied to the material before compressive failure of the die liner 4a occurs. The reason for this, though not fully understood, is believed to be that the axial liner force  $F_3$  opposes the axial components of the essentially radial force  $F_2$ , thereby preventing the separation of the liner as in the prior art method described above. By preventing this separation, or axial tensile failure, the catastrophic combination of compressive and axial tensile failure of the die liner 4a is prevented.

Hence, by applying axial compression to a die liner 4a, the walls of which are supported by a support sleeve 5a, material 6a within that liner 4a can be compressed at pressures greater than normally possible.

The preferred material for the die liner 4a is graphite. This is at least because of its lubricating quality, ease of machining, low cost, and relative chemical inertness under many conditions. Graphite is also capable of being used at very high temperatures, provided that the operation is carried out in a vacuum, or in an inert atmosphere free of oxygen and moisture. However, the general method described herein is not limited to the use of graphite as a die liner. Any material that is presently in use or may be used in the future as a die liner can be employed in the practice of the novel method of pressing materials described herein. Examples of materials other than graphite that may be used as a die liner are metal nitrides and carbides such as boron nitride or boron carbide; and ceramic oxide materials such as alumina, magnesia, and zirconia.

The support sleeve 5a, the rams 2a and 3a, and the plug 11 can be made of any materials that are capable of withstanding the stresses upon them. For example, the support sleeve 5a, rams 2a and 3a, and the plug 11 may be made of essentially any of the materials used in the conventional presses and hot-presses as support sleeves or compression rams, or of any materials that may be used therefor in the future. Examples of materials presently in use include molybdenum alloys, stainless steel, chrome-nickel alloys, and tungsten carbide.

Any of the conventional means for heating the die and material contained therein may be used including resistance and induction heating of the die liner or material therein.

The method is most applicable to the pressure compacting and pressure sintering of powders which melt at relatively high temperatures, e.g., ceramics, ferrites, or other refractory materials. Compaction of such powders normally requires high pressures and temperatures. However, the general method is applicable in any pressure compacting, pressure sintering, or pressure molding process. Examples of materials that may be compacted or pressure sintered by this method to form uniform compact bodies are given in the following table.

| Class of materials:              | Examples                                                                                                              |
|----------------------------------|-----------------------------------------------------------------------------------------------------------------------|
| Semiconductive compounds         | CdS, ZnS, CdTe, ZnSe, PbTe, GaAs, GaSb, InSb.                                                                         |
| Elemental semiconductors         | Ge, Si.                                                                                                               |
| Ferrites                         | Mn-Zn ferrite, Li-ferrite, yttrium iron garnet.                                                                       |
| Oxide ceramics                   | Al <sub>2</sub> O <sub>3</sub> , SiO <sub>2</sub> , BeO, ZrO <sub>2</sub> , MgO, TiO <sub>2</sub> , UO <sub>2</sub> . |
| Ferroelectrics                   | BaTiO <sub>3</sub> , PbZrO <sub>3</sub> , Pb (Zr, Ti)O <sub>3</sub> , NaTaO <sub>3</sub> , NaNbO <sub>3</sub> .       |
| Superconducting materials        | Nb-Sn alloys.                                                                                                         |
| Refractory carbides and nitrides | ZrC, HfC, BN, UC <sub>2</sub> .                                                                                       |
| Other inorganic compounds        | MgF <sub>2</sub> , LiF, CaF <sub>2</sub> , LaF <sub>3</sub> .                                                         |
| Metals                           | Ni, W, Ti.                                                                                                            |

The method is also applicable to pressure bonding of various materials, and to pressure molding of self-lubricating composites from metals and solid lubricants. Typical ranges of pressure and temperature for the compression of inorganic powders by the novel method are 10,000 to 100,000 pounds per square inch pressure at temperatures of from about room temperature to about 2500° C.

*Example 1.*—A die and ram assembly of the type shown in FIG 2 having two cylindrical rams 2a and 3a of about 1/2 inch in diameter and graphite liner 4a with a wall about 3/16 inch thick is employed. The plug is screwed down with a wrench so as to apply a torque of 42 foot-pounds to the plug 11. A value of about 17,000 p.s.i. of axial liner pressure is calculated from this torque. The lower ram 2a is introduced into the liner 4a. A measured quantity of gallium arsenide powder is then placed in the liner 4a. The upper ram 3a is introduced into the liner 4a and advanced toward the lower ram 2a thereby compressing the powder between the rams 2a and 3a. The pressure is maintained for about one hour with the powder heated to about 900° C. Then, the upper ram 3a is retracted from the liner 4a and the compressed material is removed from the liner 4a. Ram pressures of at least up to about 80,000 p.s.i. can be applied using the novel method. Prior methods using dies of the type shown in FIG 1 with the same liner 4a and ram 2a and 3a dimensions can apply pressures to the powder of only about 25,000 p.s.i. at 900° C.

*Example 2.*—Using the die and ram assembly described in Example 1 and following the same general procedure as described therein, calcium fluoride powder can be pressed with applied pressures of at least about 50,000 p.s.i. at a temperature of about 1,000° C. The prior methods using dies of the type shown in FIG 1 having the same liner and ram dimensions can only be used at applied pressures to the powder of up to about 15,000 p.s.i. at 1,000° C.

What is claimed is:

1. A method for pressing particulate material to form a compacted unitary body therefrom including the steps of:
  - (a) placing the material to be pressed into a die, said die comprising a support sleeve and a liner within said sleeve, said support sleeve supporting said liner when outwardly directed radial pressure is present on said liner;
  - (b) compressing said liner in the axial direction;
  - (c) compressing said material within said die so as to form a unitary body therefrom while maintaining compression on said liner in the axial direction of sufficient magnitude to prevent failure of said liner.
2. A method for pressing material as described in claim 1 including heating the material to be compressed so that said material will be at a prescribed elevated temperature during the step of compressing said material.

3. A method for pressing material as described in claim 1 wherein said liner is made of graphite.

4. A method for pressing material as described in claim 3 including the step of removing essentially all of the oxygen and moisture from the atmosphere surrounding said material to be compressed.

5. A method for pressing materials as described in claim 3 wherein said materials to be compressed are powders of inorganic compounds, said compounds being compressed at pressures in the range between 10,000 and 100,000 pounds per square inch, while at temperatures of from about room temperature to about 2500° C.

2,909,417 10/1959 Osenberg ----- 51-293  
3,230,286 1/1966 Bobrowsky ----- 264-120

## OTHER REFERENCES

5 Advanced Mechanics of Materials, 2nd edition, F. B. Seely and J.O. Smith, John Wiley & Sons, New York, 1952, pages 301 and 309.

10 ROBERT F. WHITE, *Primary Examiner.*

J. R. HALL, *Assistant Examiner.*

## References Cited

## UNITED STATES PATENTS

|           |         |             |         |    |         |
|-----------|---------|-------------|---------|----|---------|
| 3,154,006 | 10/1964 | Novak ----- | 52-223  | 15 | 264-338 |
| 3,258,514 | 6/1966  | Roach ----- | 264-125 |    |         |

## U.S. CL. X.R.